

## UNITED STATES PATENT OFFICE

1,984,636

## MACHINABLE STAINLESS CASTING

Frank A. Fahrenwald, Chicago, Ill.

No Drawing. Application June 26, 1933,  
Serial No. 677,761

1 Claim. (Cl. 75—1)

This invention relates to machinable stainless or rustless alloy-castings or articles, for example, pipes and tubes, together with valves, fittings, faucets and the like used in connection therewith; also household utensils, such as kettles or pans; decorative objects such as plaques, nameplates and the like; and various ornamental forms requiring a surface stable under atmospheric conditions.

10 This alloy has proved particularly adaptable to the manufacture of parts for centrifugal and reciprocating pumps, and for fittings and valves such as are employed in the handling of corrosive liquids in various industries. Materials heretofore available for such purposes have been cast iron, bronze, various forms of plated ware, and, more latterly, some of the so-called stainless alloys containing, for instance, 18% of chromium and 8% of nickel.

20 A great demand has existed for a nickel-chromium or high chromium type of casting for the above-named and similar uses, but due to the very great difficulty encountered in production, alloys of compositions known heretofore have not 15 been commercially available for these applications. The prime requisites for such an alloy, in addition to surface stability, are ease of casting in the foundry and ease of machining or otherwise working, to adapt the casting for some specific use.

It has heretofore been claimed that for a casting to have corrosion resisting qualities and to be easily machinable, its carbon content must be low, and this is reiterated throughout the prior art. In my own experiments, undertaken to produce castings of these types, I have employed higher percentages of chromium and higher percentages of carbon and whereas I found at first, in common with the claims of the prior art, that 35 when the chromium content or carbon content is increased to only a medium degree above the low carbon ranges constantly heretofore specified, very great hardness, fragility and unmachinability resulted, yet if the chromium and carbon are increased far above that previously employed, the alloys again reach a machinable range in composition and besides take on production characteristics which render them producible in forms 40 hitherto considered utterly impossible.

Whereas the older forms of stainless alloys are tough and difficult to machine, my new alloy can be cut, drilled or filed with extreme ease and, while it lacks the ductility or toughness of the low 45 carbon alloys, I have been enabled to render it

sufficiently strong and tough for all of the purposes hereinbefore enumerated.

All low carbon nickel-chromium alloys have a high shrinkage from liquid to solid and have a long range between solidness and liquidness during solidification, with resulting proneness to develop cracks and shrink holes during casting.

5 The older low carbon alloys are of high melting point, requiring expensive refractory molding sands; whereas, my new alloy is of much lower melting point and castings can be made in cheap sands ordinarily employed for gray iron castings.

Likewise, regarding the requirement for a low carbon content and for stainless qualities in the older types of alloys, I have found that high carbon percentages may be employed providing the 10 chromium content is increased proportionately.

The basis of my new alloy casting is a combination of iron, chromium and carbon—the chromium varying between 30 and 40% and the 20 carbon between 1.25 and 2.75%, to which, for reasons hereinafter described, I make nickel additions varying from  $\frac{1}{2}$  of 1% to 15%; one typical formula within these limits being chromium 35%; nickel 2%; carbon 2%; and the balance 25 iron, which has been found to answer well the conditions encountered in centrifugal pumps. Another formula, and one found resistant to 10% sulphuric acid, is chromium 34.9%; nickel 9% and carbon 1.9%. A straight chromium-iron 30 casting containing 36.4% chromium and 2.20% carbon was found to possess the qualities of great fluidity in casting and machinability when cast, but possessed the unfortunate characteristic of great brittleness, besides lacking required resistance to corrosion. But I have found that the brittleness is very rapidly eliminated by small 35 additions of nickel; whereas, the resistance to corrosion is at the same time thereby tremendously increased. Nickel-free castings of this type are so brittle as to render handling during production and machining quite difficult, but the addition of even  $\frac{1}{2}$  of 1% of nickel overcomes this deficiency; whereas 10% nickel renders the 40 castings so tough that they can be readily straightened without heating to correct warpings introduced during a casting operation. Likewise, the higher nickel alloys are progressively more 45 immune to corrosion. But more than 15% does not seem to improve the castings either physically or chemically to a degree sufficient to justify the greatly increased cost.

From my new alloy I have produced pans and hollow containers up to ten inches in diameter of a wall thickness less than one-eighth of an inch.

5

10

15

20

25

30

35

40

45

50

55

and long thin rails and the like up to six feet in length with only five-sixteenths of an inch metal thickness.

Very intricate designs can be made from my alloy by the process of casting, and a very fine perfect surface can be produced. In contradistinction to the previously known nickel-chromium alloys with low carbon content which are very difficult to cast in many shapes or sections,

10 I have found that this new high carbon, high chromium base alloy containing nickel can be cast into practically any shape or design possible with brass or bronze.

The new alloy is very resistant to sulphuric acid, practically immune to nitric and organic acids, and immune to the action of all of the commoner alkaline solutions. It is completely immune against atmospheric corrosion and will take a highly polished finish which retains its

15 luster equally as well as does the previously employed low carbon, low chromium stainless alloy.

Castings made from this alloy can be manufactured from raw materials costing less than one-half as much as castings of the low carbon

type. Due to its lower melting point and protection against oxidation, my new alloy can be melted in fuel fired furnaces at a cost reduced by 75% as compared with electric furnaces. Foundry production costs are far lower because of the cheaper sands permissible, higher yield, more perfect castings and easy finishing or machining operations which, in thin as well as thick sections, compare favorably with those of cast gray iron, in that they respond to ordinary finishing tools in the average machine shop manned with common skilled labor.

10 The formulas given are in terms of essential ingredients only. Percentages of molybdenum, tungsten, copper, manganese, etc. frequently encountered in iron or iron alloy castings may be present without departing from the spirit of the invention.

15 I claim:

A machinable stainless alloy casting consisting of iron, with chromium about 35%, nickel from  $\frac{1}{2}$  of 1% to 15%, and carbon around 2%.

FRANK A. FAHRENWALD.